

1

2,758,091

## LUBRICATING COMPOSITIONS

William Cyril Webber, New Malden, England, assignor to Shell Development Company, Emeryville, Calif., a corporation of Delaware

No Drawing. Application April 28, 1952,  
Serial No. 284,807

Claims priority, application Great Britain  
October 28, 1947

8 Claims. (Cl. 252—49.9)

This invention relates to extreme pressure lubricants capable of withstanding high pressures at elevated temperatures under severe and adverse operating conditions. More specifically, this invention pertains to extreme pressure lubricants which are non-corrosive and stable, due to the presence therein of relatively minor amounts of certain novel additives.

Natural and/or synthetic lubricants, per se, are not capable of withstanding extreme pressures at high temperatures, high speeds and severe loading conditions generally encountered in present day lubrication of various internal combustion engines, transmission devices, hypoid gears, as well as in metal fabrication, such as in cutting and drawing operations. Under such conditions of lubrication, the protective film formed by the lubricant between contacting surfaces, so as to prevent direct metal-to-metal contact, breaks down or ruptures, thereby causing seizure or even welding of metal parts; this results in serious damage to the elements being lubricated. To overcome this serious weakness generally inherent in undoped lubricants, extreme pressure agents are usually added; these agents form protective films between contacting surfaces and possess, among their properties, the function of imparting film strength and oiliness to the lubricants, thus preventing their breakdown and rupture under the above-described lubricating conditions.

The action of extreme pressure agents is largely a physicochemical phenomenon, and this accounts primarily for their effectiveness as extreme pressure agents. These agents, in addition to increasing the film strength of lubricants, react with the contacting metal surfaces, forming thereon a protective coating or film of great strength and thermal stability. This tenaciously adhering adsorbed protective film not only reduces friction between moving parts, such as those encountered in internal combustion engines, but also acts as an impermeable film which prevents corrosive acids and other contaminants from attacking the metal surfaces. To be effective, therefore, extreme pressure agents must, to a degree, be reactive with contacting surfaces and form thereon a protective film which prevents welding of moving parts and aids lubrication. Since the reaction is normally between the additives in the lubricants and the contacting surfaces at elevated temperatures of around about 500° C. and higher, the performance of a given lubricant must depend upon its composition, the composition of the contacting surfaces being lubricated, and the conditions to which the lubricant and the surfaces are subjected.

Although extreme pressure additives, in order to be effective, should be reactive with contacting surfaces, this reactivity should not be corrosive to the reactive surface. This is generally a serious drawback of known extreme pressure agents, for serious damage to metal surfaces, particularly in the case of alloy bearings, might result. Such additives should also not tend to promote oxidation which generally prompts formation of corrosive acidic materials, sludge, lacquer and varnish; this

2

in turn results in sticking and fouling of movable engine parts.

Numerous compounds and mixtures of compounds have been proposed and tried as extreme pressure agents for lubricants, the best of which have only moderately improved the extreme pressure properties of the lubricant, and even this generally at the expense of increased corrosiveness and instability of the lubricant.

It is an object of the present invention to provide an improved extreme pressure type lubricant capable of effective lubrication under high pressures at elevated temperatures and adverse operating conditions. Still another object of this invention is to provide an improved, stable, sludge free, non-corrosive extreme pressure lubricant. Also, it is an object of this invention to provide an improved extreme pressure lubricant by addition to any lubricating carrier or base a minor amount of a novel reaction product of this invention. Still another object is to form an improved non-corrosive extreme pressure additive. Other objects of this invention will appear as the description proceeds.

Broadly stated, this invention is directed to improved lubricants containing a minor amount of a trihalomethylarylcarbonyl phosphorus compound selected from the group consisting of phosphite, phosphate, and phosphonate esters, and also to the improving agents themselves.

The compounds are suitably represented by the formula



and the other chalcogen analogues (S, Se, Te) thereof, wherein  $n$ ,  $m$  and  $p$  are whole numbers from 0 to 1, with  $n+p$  being at least 1, and  $n+m+p$  being at least 2, and A is a trihalomethylarylcarbonyl radical, e. g., 1-trichloromethyl-1-phenyl-carbonyl, and the R's are independently selected hydrogen atoms or organic radicals which are residues of alcohols and phenols of the formula  $\text{ROH}$ , preferably hydrocarbyl radicals, especially alkyl radicals, of 1 to 8 carbon atoms. The halogen atoms in A are preferably selected from chlorine and bromine.

The aryl radical may be nuclearly substituted with substituent groups such as lower alkyl, aryl, nitro, amino, hydroxyl, etc., particularly the para-nitro group.

The compounds can be prepared by forming 2,2,2-trihalo-1-arylethanol in accordance with the method of Chattaway and Muir (Journal of the Chemical Society 1934, p. 701) and reacting said compound with a suitable phosphorus compound such as a phosphite triester.

As an illustrative example, the following method was employed in preparing diethyl (1-phenyl-2,2,2-trichloroethyl) phosphite.

About 1 mol of benzene and 3 mols of chloral hydrate were reacted by the method of Chattaway and Muir so as to yield 2,2,2-trichloro-1-phenylethanol. About 1 mol of this material was treated with about 1 mol of triethyl phosphite in benzene using trichloroacetic acid as a catalyst. After the reaction was complete, the benzene was removed by distillation and the unreacted triethyl phosphite removed by distillation in vacuo at 100° C. The final product was diethyl (1-phenyl-2,2,2-trichloroethyl) phosphite.

The following are other specific compounds exemplifying the compounds defined broadly above:

65 Dibutyl (1-phenyl-2,2,2-trichloroethyl) phosphite  
Dicsresyl (1-phenyl-2,2,2-trichloroethyl) phosphite  
Dicyclohexyl (1-phenyl-2,2,2-trichloroethyl) phosphite  
Diethyl (1-phenyl-2,2,2-trichloroethyl) phosphate  
Diethyl (1-phenyl-2,2,2-tribromoethyl) phosphate  
70 Ethyl butyl (1-phenyl-2,2,2-dichloromonobromoethyl) phosphate

Ethyl (1-phenyl-2,2,2-trichloroethyl) ethanephosphonate  
Octyl (1-phenyl-2,2,2-trichloroethyl) octanephosphonate  
Cresyl (1-phenyl-2,2,2-trichloroethyl) methanephosphonate  
Butyl (1-phenyl-4,4,4-trichlorobutyl) butanephosphonate  
Ethyl (1-naphthyl-2,2,2-trichloroethyl) ethanephosphonate  
Ethyl (1-phenyl-2,2,2-trichloroethyl) acid phosphite  
Ethyl (1-phenyl-2,2,2-trichloroethyl) acid phosphate  
Diethyl [1-(4-nitrophenyl)-2,2,2-trichloroethyl] phosphite  
Dicresyl [1-(4-chlorophenyl)-2,2,2-trichloroethyl] phosphite  
Diethyl (1-phenyl-2,2,2-trichloroethyl) thiophosphite  
Dicresyl (1-phenyl-2,2,2-trichloroethyl) thiophosphite  
Diethyl (1-phenyl-2,2,2-trichloroethyl) selenophosphite  
Diethyl (1-phenyl-2,2,2-trichloroethyl) telurophosphite  
Diethyl (1-phenyl-2,2,2-trichloroethyl) thiophosphate  
Diethyl (1-phenyl-2,2,2-trichloroethyl) trithiophosphite  
Diethyl (1-phenyl-2,2,2-trichloroethyl) trithiophosphate  
Diethyl (1-phenyl-2,2,2-trichloroethyl) triseleno phosphite  
Diethyl (1-phenyl-2,2,2-trichloroethyl) dithiophosphite  
Dibutyl (1-phenyl-2,2,2-trichloroethyl) trithiophosphite

Of the extreme pressure additives within the ambit of this invention, those are preferred which are soluble in the lubricant to an extent sufficient to give the compounded lubricant desired extreme pressure properties. It is possible, however, to produce excellent extreme pressure lubricants by dispersing the additives in the lubricant in the form of a stable colloidal suspension; thus, even those additives which are not readily soluble in the base lubricant can be employed. Suitable stabilizing and solubilizing agents may be added, such as long chain fatty alcohols having 8 to 20 carbon atoms, organic sulfonates, and the like.

In general, good results can be obtained by addition of the subject additives to a base lubricant in an amount of from a fraction of 1% up to 10%, the preferred range being from 0.1% to about 5% by weight.

The base for additives of this invention can be any natural or synthetic materials having lubricating properties. Thus, the base may be a hydrocarbon oil obtained from a paraffinic, naphthenic, Mid-Continent or Coastal stock and/or mixtures thereof. The viscosity of these oils may vary over a wide range such as from 100 SUS at 100° F. to 2000 SUS at 100° F. These oils may be refined by any of the well known processes. The hydrocarbon oils may be blended with fixed oils, such as castor oil, lard oil, and the like, and/or with synthetic lubricants, such as polymerized olefins, copolymers of alkylene glycols and alkylene oxides, organic esters (e. g., 2-ethyl hexyl sebacate, dioctyl phthalate, trioctyl phosphate), polymeric tetrahydrofuran, or polyalkyl silicone polymers, e. g., dimethyl silicone polymer, and the like. If desired, the synthetic lubricants may be used as the sole base lubricant or admixed with fixed oils and derivatives thereof.

General formulation of compositions of this invention can be represented by:

| Amount (per cent by weight)                                                                 |                   |
|---------------------------------------------------------------------------------------------|-------------------|
| Organic phosphorus compound of this invention containing at least one CX <sub>3</sub> group | 0.1 to 10 (0.1-5) |
| Other additives, such as sulfonates, corrosion inhibitors, detergents, etc.                 | 0 to 2 (0.01-0.5) |
| Base lubricant (natural and/or synthetic)                                                   | Balance           |

Compositions of this invention were evaluated as extreme pressure agents by use of the Four-Ball Tester similar in principle to the Boerlage apparatus described in the magazine "Engineering," volume 136, July 13, 1933. This apparatus comprises four steel balls arranged in a pyramid formation. The top ball is rotated by spin-

des against the three bottom balls which are clamped in a stationary ball holder. The balls are immersed in the compositions to be tested. Tests were run with undoped mineral oil and with 1% by weight of a lubricant of this invention as indicated in the table below under various loads and the wear at these loads was measured. The fixed conditions under which the test were conducted are:

Speed: 1500 R. P. M.  
Test duration: 60 seconds  
Temperature: Ambient  
Hoffmann steel balls

Lubricants of this invention were also tested on the I. A. E. 3 1/4 in. centres gear rig. The results obtained are summarized in the table below:

I. A. E. 3 1/4 centres:  
Pinion speed 2000 R. P. M.  
Gears 15/16 tooth

The gear material was En 39 and En 34

Base oil: mineral oil

| Additive Conc., percent wt. | Additive                                          | Four-Ball Machine Wear Score Diam. at 140 kg. Load   |
|-----------------------------|---------------------------------------------------|------------------------------------------------------|
|                             |                                                   | 3.69 mm. 0.70 mm.                                    |
| None                        | diethyl (1-phenyl-2,2,2-trichloroethyl) phosphite |                                                      |
| Additive Conc., percent wt. | Additive                                          | I. A. E. 3 1/4" Gear Rig Scuffing Load (lbs.) 50° C. |
|                             |                                                   | 17. 145.                                             |

Products of this invention can be combined with other additives in lubricants, such as blooming agents, pour point depressants or viscosity improvers, extreme pressure agents, anti-foaming agents, and the like. Among the specific additives which can be used are oil-soluble detergents which include oil-soluble salts of various bases with detergent forming acids. Such bases include metal as well as organic bases. Metallic bases include those of the alkali metals and of Cu, Mg, Ca, Sr, Ba, Zn, Cd, Al, Sn, Pb, Cr, Mn, Fe, Ni, Co, etc. Organic bases include various nitrogen bases as primary, secondary and tertiary amines and quaternary ammonium bases.

Examples of detergent forming acids are the various fatty acids of, say, 10 to 30 carbon atoms, wool fat acids, paraffin wax acids (produced by oxidation of paraffin wax), chlorinated fatty acids, resin acids, aromatic carboxylic acids including aromatic fatty acids, aromatic hydroxy fatty acids, paraffin wax benzoic acids, various alkyl salicylic acids, phthalic acid monoesters, aromatic keto acids, aromatic ether acids, diphenols as di-(alkylphenol) sulfides and disulfides, methylene bis alkyl phenols; sulfonic acids such as may be produced by treatment of alkyl aryl hydrocarbons or high boiling petroleum oils with sulfuric acid; sulfuric acid mono-esters; phosphoric, arsonic and antimony acid mono and diesters, including the corresponding thiophosphoric, arsonic and antimony acids; phosphonic acids and the like.

Additional detergents are the alkaline earth phosphate diesters, including the thiophosphate diester; the alkaline earth diphenolates, specifically the calcium and barium salts of diphenol mono and poly sulfides.

Non-metallic detergents include compounds such as the phosphatides, such as lecithin and cephalin, certain fatty oils as rapeseed oils, volatilized fatty or mineral oils and the like.

An excellent metallic detergent for the present purpose

is the calcium salt of oil-soluble petroleum sulfonic acids. This may be present advantageously in the amount of about 0.025% to 0.2% sulfate ash. Also alkaline metal salts of alkyl phenol-aldehyde condensation reaction products are excellent detergents.

Antioxidants comprise several types, for example, alkyl phenols such as 2,4,6-trimethyl phenol, pentamethyl phenol, 2,4-dimethyl-6-tertiary-butyl phenol, 2,4-dimethyl-6-octyl phenol, 2,6-ditertiary-butyl-4-methyl phenol, 2,4,6-tri-tertiary-butyl phenol and the like; amino phenols as benzyl amino phenols; amines such as dibutyl-phenylene diamine, diphenyl amine, phenyl-beta-naphthylamine, phenyl-alpha-naphthylamine, dinaphthyl amine.

Corrosion inhibitors or anti-rusting compounds may also be present, such as dicarboxylic acids of 16 and more carbon atoms; alkali metal and alkaline earth salts of sulfonic acids and fatty acids; organic compounds containing an acidic radical in close proximity to a nitrile, nitro or nitroso group (e. g., alpha cyano stearic acid).

Additional ingredients may comprise oil-soluble urea or thiourea derivatives, e. g., urethanes, allophanates, carbazides, carbazones, etc.; polyisobutylene polymers, unsaturated polymerized esters of fatty acids and mono-hydric alcohols and other high molecular weight oil-soluble compounds.

Depending upon the additive used and conditions under which it is used, the amount of additive used may vary from 0.1 to 2% or higher. However, substantial improvement is obtained by using amounts ranging from 0.1 to 0.5% in combination with polyhalogen containing organic carbonyl compound and organic thiol, selenol and/or tellurol compound reaction products of this invention.

The novel phosphorus products of this invention, in addition to being excellent lubricating oil improving agents, are potent oxidation inhibitors for fuels, natural and synthetic rubber, wax coating compositions and other organic materials.

It is to be understood that while the features of the invention have been described and illustrated in connection with certain specific examples, the invention, however, is not to be limited thereto or otherwise restricted, except by the prior art and the broad scope of the disclosed invention.

This application is a continuation-in-part of my co-

pending application Serial No. 55,043 filed October 18, 1948, which has matured into U. S. Patent 2,599,794.

I claim as my invention:

- 5 1. A lubricating composition consisting essentially of a major amount of a lubricating oil and a minor amount sufficient to impart extreme pressure properties thereto, of a dihydrocarbyl trihalomethyl-1-arylalkyl phosphite.
- 10 2. A composition of claim 1 but wherein the halo element is chlorine.
- 15 3. A composition of claim 2 but wherein the lubricating oil is a mineral lubricating oil.
4. A lubricating composition consisting essentially of a major amount of a mineral lubricating oil and a minor amount sufficient to impart extreme pressure properties thereto of a dialkyl trichloromethyl-1-aryl-alkyl phosphite.
- 20 5. A lubricating composition consisting essentially of a major amount of a mineral lubricating oil and a minor amount sufficient to impart extreme pressure properties thereto of a dialkyl trichloromethyl-1-phenyl-alkyl phosphite.
- 25 6. A lubricating composition consisting essentially of a major amount of a mineral lubricating oil and a minor amount sufficient to impart extreme pressure properties thereto of diethyl (1 - phenyl - 2,2,2 - trichloroethyl) phosphite.
- 30 7. A lubricating composition consisting essentially of a major amount of a mineral lubricating oil and a minor amount sufficient to impart extreme pressure properties thereto of dibutyl (1 - phenyl - 2,2,2 - trichloroethyl) phosphite.
- 35 8. A lubricating composition consisting essentially of a major amount of a mineral lubricating oil and a minor amount sufficient to impart extreme pressure properties thereto of dicresyl (1 - phenyl - 2,2,2 - trichloroethyl) phosphite.

#### References Cited in the file of this patent

#### UNITED STATES PATENTS

|    |           |               |               |
|----|-----------|---------------|---------------|
| 40 | 2,432,095 | Frey          | Dec. 9, 1947  |
|    | 2,520,393 | Fletcher      | Aug. 29, 1950 |
|    | 2,573,568 | Harman et al. | Oct. 30, 1951 |
|    | 2,597,534 | Schrader      | May 20, 1952  |

#### FOREIGN PATENTS

|    |         |           |               |
|----|---------|-----------|---------------|
| 45 | 142,944 | Australia | Aug. 16, 1951 |
|----|---------|-----------|---------------|